

1

3,711,366

**DIGESTING LIGNOCELLULOSIC MATERIAL WITH SODIUM HYDROXYMETHYLSULFONATE**

Junzo Nakano, Yuichiro Sumi, and Makoto Nagata, Tokyo, Japan, assignors to The Kokusaku Pulp Industry Co., Ltd., Tokyo, Japan

No Drawing. Continuation-in-part of application Ser. No. 657,526, Aug. 1, 1967. This application Sept. 22, 1970, Ser. No. 74,469

Claims priority, application Japan, Aug. 3, 1966,

41/50,503

Int. Cl. D21b 1/16

U.S. Cl. 162—24

5 Claims

**ABSTRACT OF THE DISCLOSURE**

Improvement in a process for manufacturing high yield pulp in which cooking treatment and mechanical defibration for lignocellulosic material are combined, said cooking treatment being carried out in alkaline condition employing a sulfomethylation agent which is produced from admixing sodium sulfite and/or sodium bisulfite, formaldehyde and water, said mechanical defibration being carried out either before or after the cooking.

This application is a continuation-in-part of the pending Ser. No. 657,526, filed on Aug. 1, 1967, now abandoned.

Various processes for producing high yield pulp have been suggested. High yield pulp has already been obtained by groundwood, chemigroundwood and semichemical pulping processes but the high yield pulp so produced contains more lignin than the conventional chemical pulp and, therefore, beating and refining have little effect, no or less fibrillation results, and the strength of the paper produced therefrom is relatively low. Thus, a process for making high yield pulp which is easily beaten and refined to produce a high strength paper is desired.

A sulfite process for red pine native to Japan employing formaldehyde as additive was disclosed in the Journal of the Chemical Society of Japan, Industrial Chemistry Section 54, 195 and 397, 151 and 56, 277. Phenolic compounds in the raw material reacted with the formaldehyde in the sulfite cooking liquor and condensation reaction, which was considered to cause burnt cook, between the phenolic compounds and lignin was avoided. This process was useful for cooking red pine chips containing heart wood. E. Adler and L. Stockman disclosed in the Svensk Papperstidning 54, 477 that wood was subjected to chemical pulping process using sulfite cooking liquor containing formaldehyde where burnt cook was observed and it was considered that pulping is impossible.

Sodium sulfite or sodium bisulfite, formaldehyde and water are reacted to obtain sodium hydroxymethylsulfonate by the following reactions:



In the case of Reaction 1, it is recognized that about 10% by weight of the original sodium sulfite is converted into sodium hydroxymethylsulfonate under the conditions described hereinafter in the examples; the resulting aqueous solution has a pH range of about 12.4 and 12.7. The aqueous solution contains sodium sulfite, formaldehyde, sodium hydroxymethylsulfonate and sodium hydroxide.

In Reaction 2, the sodium bisulfite is quantitatively converted into sodium hydroxymethylsulfonate and the resulting solution shows a pH of about 4.5. An alkali should be added to maintain the pH value in near neutral to alkaline condition, i.e. at a pH from 5.7 to 13.7.

2

In the case of Reaction 1, some of the  $\text{Na}_2\text{SO}_3$  added is converted into  $\text{HOCH}_2\text{SO}_3\text{Na}$  and the remaining is maintained in its original state, and, in the case of Reaction 2, all of the  $\text{NaHSO}_3$  added is converted into  $\text{HOCH}_2\text{SO}_3\text{Na}$ ; if  $\text{Na}_2\text{SO}_3$ ,  $\text{NaHSO}_3$ ,  $\text{HCHO}$  are employed, the following reaction would occur:



Thus, the composition of the liquid formed is complicated and it is difficult to analyze the composition by a conventional method. It is, however, possible to measure the pH value from which the amount of  $\text{NaOH}$  may be interpreted. Thus, the equilibrium values of the constituents can be estimated from the degree of formation of  $\text{NaOH}$ . It is necessary to adjust the pH value of the liquid to the range abovementioned.

The sulfomethylation agent produced as above reacts with lignin. Details of the reaction have not been confirmed, but it seems that:

- (1) addition reaction of formaldehyde and the aromatic ring in lignin occurs to form an alcoholic hydroxy group; subsequently the hydroxy group is sulfonated with sodium sulfite or bisulfite to form sulfomethylated lignin;
- (2) ortho position to phenolic hydroxy group in lignin is directly sulfomethylated with sodium hydroxymethylsulfonate; and
- (3) in addition to the above, the side chain portion in lignin may also be sulfomethylated.

Lignocellulosic materials including soft and hard wood, straw, bamboo, grass and like are cooked by the aqueous solution when the lignin is sulfomethylated according to the above reactions. Of course, side-reactions occur, for example, between other chemicals such as sodium sulfite, sodium bisulfite and sodium hydroxide and non-cellulosic materials such as lignin, hemicellulose and others.

In cooking, that part of the lignin which does not combine with carbohydrates is dissolved in the cooking liquor, while the lignin that combines with the carbohydrates is not dissolved but is converted into a hydrophilic and soft state by sulfomethylation. The resulting cooked material is easily defibrated mechanically without fiber shortening and specific fiber damage.

Pulp so treated contains a larger amount of lignin than the conventional chemical pulps, so the yield of pulp according to this invention is high. Furthermore, since the lignin is in a hydrophilic and soft state, fiber containing such lignin is easily fibrillated by beating and refining.

Alternatively, lignocellulosic material predefibrated by, for example, grinder and refiner can then be cooked with the aqueous sulfomethylation agent solution.

One way of carrying out the present invention is to carry out the cooking under elevated pressure and temperature employing a large amount of the aqueous sulfomethylation agent solution; this is similar to "liquid phase cooking process." Another way is to immerse the lignocellulosic material in the cooking liquor, then remove excess liquor, and subsequently, heat the lignocellulosic material by steam as in the conventional "vapor phase cooking process." In this case, the cooking time and liquid ratio would be decreased.

The cooking conditions employed in this invention are a temperature of about 100° C. to 190° C., a pressure of about 0.5 kg./cm.<sup>2</sup> gauge to 16 kg./cm.<sup>2</sup> gauge, and the molar ratio of formaldehyde to sulfite and/or bisulfite of 0.8 to 1.2, and, in the liquid phase cooking, a time of 20 minutes to 5 hours, a liquid ratio of 2 to 20, preferably 3.5 to 8 and a concentration of cooking liquor of about 5 to 30% by weight calculated as  $\text{SO}_2$  for lignocellulosic

material and, in the vapor phase cooking, a time of few minutes to one hour, a liquid ratio of 1.0 to 4.0 and a concentration of 2 to 15% are employed. The pH of the cooking liquor is an important factor; it is desirable to maintain near neutral to alkaline condition throughout the cooking treatment. It has been found that the yield of pulp is from about 70 to 90% by weight for raw material.

The term "liquid ratio" is conventionally used in the pulp industry to define the following relationship:

#### Liquid ratio

$$= \frac{\text{the volume of the liquor added}}{\text{the oven-dried weight of wood chip (kg.)} + \text{water in the wood chip (l.)}}$$

When lignocellulosic material is processed according to this invention the pH value of the cooking liquor decreases as the reaction proceeds, because an acid is produced from the lignocellulosic material and sodium hydroxide is consumed by the reaction. However, it is desirable to bring the pH value of the cooking liquor to a pH of 10.9 to 13.7, more suitably 11.9 to 12.7 when cooking treatment is started, and the end point will be from 10.6 to 5.7, more suitably 9.6 to 6.7. Therefore, an alkali should be added to the cooking liquor produced from sodium bisulfite and formaldehyde to bring the pH within the range mentioned above. In any case, care should be taken throughout the cooking treatment to avoid an extremely acid condition.

The pulp produced in accordance with this invention has a brightness of 47% to 53% and a light yellow colour. It is useful as unbleached pulp, but, if desired, it can be bleached with hydrogen peroxide to increase brightness to about 70%.

Preferred embodiments of the present invention will be given by way of examples in which the novel process is successfully carried out.

#### EXAMPLE 1

2325 ml. of an aqueous sulfomethylation agent solution was prepared which contained 51.6 g. of sodium sulfite, 11.3 g. of formaldehyde and 11.5 g. of hydrochloric acid per liter (the molar ratio of formaldehyde to sulfite being 0.9) and had a pH of 9.4. Lignocellulosic material was immersed in the solution and the excess solution was removed at which the pH value of the solution was 8.1. The immersed material was vapor phase cooked at a temperature of 148° C. under a pressure of 4.5 kg./cm.<sup>2</sup> gauge for 8 minutes under the conditions of a liquid ratio of 1.6 and a SO<sub>2</sub> concentration of 4.1%, and then defibrated for 2 minutes at the same temperature. The pH value of the cooking solution after defibration was 3.5. The yield of pulp after defibration was 89.8%. The pulp so obtained had a freeness of 780 cc. (CSF) and even after treatment with a Lampen mill for 5 hours the freeness was 770 cc. (CSF). The decrease in freeness was extremely small. This was similar to pulp produced by the Asplund process in which lignocellulosic material was immersed in cooking liquor containing 51.5 g. of sodium sulfite per liter, after removing the excess liquor heated at temperature of 148° C. for one hour by steam and defibrated at that temperature. Both pulps were unsatisfactory for use of paper. Furthermore, wood chips were processed with a similar aqueous sulfomethylation agent solution having pH value of 5.0; the pH value after the cooking reached 2.2. The resulting pulp had a dark brown colour, so that it could not be employed for paper industry. These phenomena support the idea that an extreme acid condition throughout cooking treatment should be avoided.

#### EXAMPLE 2

Mixed chips of six kinds of hard wood native to Hokkaido, Japan, weighing 375 g. (oven dried weight was 300 g.) were evacuated. 2325 ml. of cooking liquor containing 51.6 g. of sodium sulfite and 11.3 g. of formaldehyde

per liter (the molar ratio of formaldehyde to sulfite being 0.9, a liquid ratio being 8.0 and a SO<sub>2</sub> concentration being 20.3%) and having a pH of 12.7 was added to the chips. Cooking treatment was carried out at a temperature of 150° C. under a pressure of 5 kg./cm.<sup>2</sup> gauge for 30 minutes. The pH value at end of the cooking was 7.9. The cooked chips were separated from the cooking liquor and defibrated in a Bauer laboratory disk refiner and the knots were removed therefrom. The pulp so obtained was treated by a Lampen mill and then prepared into handsheets having basis weight of 63 g./m.<sup>2</sup> by TAPPI standard.

For comparative purposes the same procedure as above was carried out, except that the cooking liquor contained only sodium sulfite. Characteristics of the pulps and strength of the handsheets are given in Table 1.

TABLE 1

|    |                                          | Present invention | Control |
|----|------------------------------------------|-------------------|---------|
| 20 | Yield of pulp after defibration, percent | 84.7              | 85.3    |
|    | Beating time (hours and minutes)         | 1.05              | 1.05    |
|    | Freeness (CSF cc.)                       | .05               | .05     |
|    | Brightness, percent                      | 44.2              | 43.2    |
|    | Breaking length (km.)                    | 6.1               | 4.5     |
|    | Burst factor                             | 3.5               | 2.3     |
| 25 | Tear factor                              | 55                | 49      |
|    | MIT folding endurance                    | 35                | 8       |

#### EXAMPLE 3

375 g. of chips and cooking liquor (the molar ratio of formaldehyde to sulfite being 0.9), the same as in Example 2, were employed. The evacuated chips were immersed in the cooking liquor until they had absorbed 480 to 500 ml. of the cooking liquor. The chips so treated were charged into a laboratory defibrator and vapor phase cooked at 148° C. under a pressure of 4.5 kg./cm.<sup>2</sup> gauge for 4 minutes under the conditions of a liquid ratio of 1.6 and a SO<sub>2</sub> concentration of 4.1%, and subsequently defibrated at the same temperature for 2 minutes. The pH value of the cooking liquor after defibration was 9.6.

The same kind of chips were vapor phase cooked and defibrated under the same conditions as in the above procedure except that the aqueous solution contained 171 g./l. of sodium sulfite and the cooking time was 60 minutes.

Handsheets were prepared as described in Example 2 from both pulps.

The characteristics of the pulps and handsheets are given in Table 2.

TABLE 2

|    |                                          | Present invention | Control |
|----|------------------------------------------|-------------------|---------|
| 55 | Yield of pulp after defibration, percent | 83.7              | 86.4    |
|    | Beating time (hours and minutes)         | 1.25              | 5.00    |
|    | Freeness (CSF cc.)                       | 330               | 450     |
|    | Brightness, percent                      | 49.8              | 47.0    |
|    | Breaking length (km.)                    | 4.5               | 2.9     |
|    | Burst factor                             | 2.5               | 1.3     |
| 60 | Tear factor                              | 50                | 36      |
|    | MIT folding endurance                    | 7                 | 2       |

#### EXAMPLE 4

65 Spruce chips were defibrated by disc refiner and the fine portion was removed, 100 g. of resulting fibers (oven dried weight being 88.7 g.) was added to 1000 ml. of aqueous solution containing 50 g. of sodium sulfite and 11 g. of formaldehyde (the molar ratio of formaldehyde to sulfite being 0.9, a liquid ratio being 11.4 and a SO<sub>2</sub> concentration being 27.7%). Cooking was carried out at a temperature of 150° C. under a pressure of 5 kg./cm.<sup>2</sup> gauge for 2 hours. The pulp thus obtained was beaten in Lampen mill and prepared into handsheets. The results are shown in Table 3.

5  
Table 3

|                                                                                        |      |
|----------------------------------------------------------------------------------------|------|
| Pulp yield (for the defibrated fiber after fine portion being removed) (percent) ----- | 89.1 |
| Beating time (hr.) -----                                                               | 1.00 |
| Freeness (CSF cc.) -----                                                               | 325  |
| Breaking length (km.) -----                                                            | 5.6  |
| Burst factor -----                                                                     | 2.8  |
| Tear factor -----                                                                      | 49   |
| MIT folding endurance -----                                                            | 59   |

## EXAMPLE 5

The procedures described in Example 4 were followed but the cooking temperature and pressure were changed to 110° C. and 1 kg./cm.<sup>2</sup> gauge. The results are shown in Table 4.

TABLE 4

|                                        |      |      |
|----------------------------------------|------|------|
| Pulp yield, percent -----              | 95.9 | 95.9 |
| Beating time (hours and minutes) ----- | 1.00 | 2.00 |
| Freeness (CSF cc.) -----               | 50   | 220  |
| Breaking length (km.) -----            | 3.9  | 4.6  |
| Burst factor -----                     | 1.5  | 2.2  |
| Tear factor -----                      | 36   | 39   |
| MIT folding endurance -----            | 4    | 9    |

## EXAMPLE 6

375 g. of the same chips as in Example 2 were added to 2325 ml. of cooking liquors, one of which contained 21.3 g. of sodium bisulfite, 25.8 g. of sodium sulfite and 11.3 g. of formaldehyde per liter and had a pH value of 11.9 (Batch I) and another of which contained 51.6 g. of sodium sulfite and 11.3 g. of formaldehyde and had a pH value of 12.7 (Batch II). The molar ratio of formaldehyde to bisulfite and sulfite (Batch I) or sulfite (Batch II) was 0.9.

The pH values of the liquors after immersing of the chips were 11.1 (Batch I) and 12.0 (Batch II).

The cooking treatment conditions were the same for Batches I and II—a temperature of 150° C. under a pressure of 5 kg./cm.<sup>2</sup> gauge for two hours under the conditions of a liquid ratio of 8.0 and a SO<sub>2</sub> concentration of 20.3%. The pH values at the end of the cooking were 6.7 (Batch I) and 7.7 (Batch II).

On the other hand, for the purpose of comparison, the procedures described above were followed but the cooking liquor contained 42.6 g. of sodium bisulfite and 11.3 g. of formaldehyde and had a pH value of 4.6 (Batch III). The pH value of the liquor after immersing of the chips was 4.6. The pH value at the end of the cooking was 3.5.

The chips separated from the cooking liquor were defibrated in a Bauer laboratory disk refiner and knots were removed therefrom. The pulps so obtained from Batches I, II and III were treated by a Lampen mill and then prepared into handsheets having a basis weight of 63 g./m.<sup>2</sup> by TAPPI standard.

The characteristic of pulps and the strength of handsheets are given in Table 5.

TABLE 5

|                                                | Batch |      |      |
|------------------------------------------------|-------|------|------|
|                                                | I     | II   | III  |
| pH of cooking liquor -----                     | 11.9  | 12.7 | 4.6  |
| Yield of pulp after defibration, percent ----- | 80.8  | 79.8 | 79.5 |
| Beating time (min.) by Lampen mill -----       | 45    | 36   | 1.5  |
| Freeness (CSF cc.) -----                       | 315   | 310  | 325  |
| Brightness, percent -----                      | 47.3  | 48.5 | 31.0 |
| Breaking length (km.) -----                    | 5.6   | 5.9  | 2.8  |
| Burst factor -----                             | 3.3   | 3.9  | 1.2  |
| Tear factor -----                              | 58    | 66   | 32   |
| MIT folding endurance -----                    | 33    | 52   | 2    |

These results show that it is desirable to maintain the pH value of cooking liquor in near neutral to alkaline condition during cooking.

## EXAMPLE 7

Spruce chips weighing 375 g. (oven dried weight being 300 g.) were evacuated. 1725 ml. of cooking liquor con-

## 6

taining 50 g. of sodium sulfite and 11.9 g. of formaldehyde per liter (the molar ratio of formaldehyde to sulfite being 1.0) and having a pH of 12.7 was added to the chips. Cooking treatment was carried out at a temperature of 160° C. under a pressure of 5.7 kg./cm.<sup>2</sup> gauge for 40 minutes under the conditions of a liquid ratio of 6.0 and a SO<sub>2</sub> concentration of 14.9%. The pH value at end of the cooking was 7.7. The cooked chips were separated from the cooking liquor and defibrated in a Bauer laboratory disk refiner. The resulting pulp was beaten and prepared into handsheet as described in Example 2.

The results are given in Table 6.

TABLE 6

|    |                                                |      |      |
|----|------------------------------------------------|------|------|
| 15 | Yield of pulp after defibration, percent ----- | 88.5 | 88.5 |
| 16 | Beating time (min.) by P.F.I. mill -----       | 2.2  | 2.6  |
| 17 | Freeness (CSF cc.) -----                       | 480  | 360  |
| 18 | Breaking length (km.) -----                    | 5.5  | 5.8  |
| 19 | Burst factor -----                             | 4.1  | 4.3  |
| 20 | Tear factor -----                              | 84   | 88   |
| 21 | MIT folding endurance -----                    | 311  | 190  |

## EXAMPLE 8

Spruce chips weighing 375 g. (oven dried weight being 300 g.) were evacuated. 1725 ml. of cooking liquor containing 30 g. of sodium sulfite and 5.7 g. of formaldehyde per liter (the molar ratio of formaldehyde to sulfite being 0.8) and having a pH of 12.5 was added to the chips (Batch IV). Cooking treatment was carried out at a temperature of 170° C. under a pressure of 7.5 kg./cm.<sup>2</sup> gauge for 80 minutes under the conditions of a liquid ratio of 6.0 and a SO<sub>2</sub> concentration of 9.0%. The pH value at end of the cooking was 7.1.

The procedures described above were followed but the cooking liquors contained 30 g. of sodium sulfite and 7.2 g. of formaldehyde (the molar ratio of formaldehyde to sulfite being 1.0) (Batch V), and 30 g. of sodium sulfite and 8.6 g. of formaldehyde (the molar ratio of formaldehyde to sulfite being 1.2) (Batch VI). In Batches V and VI, the pH values of the liquor before immersing of the chips and at the end of the cooking were 12.6 and 7.2, respectively.

The cooked chips were separated from the cooking liquor and defibrated in a Bauer laboratory disk refiner. The resulting pulps were beaten and prepared into handsheets as described in Example 2.

The results are given in Table 7.

TABLE 7

|    | Batch                                          |      |      |      |
|----|------------------------------------------------|------|------|------|
|    | IV                                             | V    | VI   |      |
| 50 | Yield of pulp after defibration, percent ----- | 81.9 | 79.6 | 81.9 |
| 51 | Beating time (min.) by P.F.I. mill -----       | 2.0  | 1.7  | 2.1  |
| 52 | Freeness (CSF cc.) -----                       | 235  | 240  | 235  |
| 53 | Breaking length (km.) -----                    | 4.1  | 4.0  | 3.8  |
| 54 | Burst factor -----                             | 3.3  | 3.3  | 3.1  |
| 55 | Tear factor -----                              | 121  | 151  | 147  |
| 56 | MIT folding endurance -----                    | 164  | 190  | 168  |

What is claimed is:

1. A process of making high yield pulp, said process comprising in combination:

(A) cooking treatment of lignocellulosic material, and

(B) mechanically defibrating lignocellulosic material, (1) said cooking treatment being carried out in an aqueous cooking liquor by means of sodium hydroxymethylsulfonate at a temperature of 100° C. to 190° C. for a period of time from a few minutes to 5 hours, at a liquid ratio of 1.0 to 20;

(i) said cooking liquor containing active pulping chemicals consisting essentially of an admixture selected from the group consisting of:

(a) sodium sulfite and formaldehyde;

(b) sodium bisulfite and formaldehyde; and

(c) sodium sulfite, sodium bisulfite and formaldehyde;

- the molar ratio of formaldehyde to sulfite, bisulfite, or sulfite plus bisulfite being 1:08 to 1.2;
- (ii) said cooking liquor having a pH of 10.9 to 13.7 at the start of cooking, and a chemical concentration of 2-30% by weight calculated as  $\text{SO}_2$  for lignocellulosic material, and a concentration of formaldehyde of 0.7-17% by weight;
- (2) said mechanically defibrating being by means of a single disc refiner; and
- (C) recovering high yield pulp.
2. A process of making pulp according to claim 1, wherein the cooking treatment is carried out in liquid phase at a temperature within the range of 100°-190° C. for a time from twenty minutes to 5 hours, at a liquid ratio of 2 to 20 and in chemical concentration of 5-30% by weight as  $\text{SO}_2$  for lignocellulosic materials. 15
3. A process of making pulp according to claim 1, wherein the cooking treatment is carried out in vapor phase at a temperature within the range of 100°-190° C., for a time from a few minutes to one hour, at a liquid 20

ratio of 1.0 to 4.0 and in concentration of 2 to 15% by weight calculated as  $\text{SO}_2$  for lignocellulosic material.

4. A process of making pulp according to claim 1, wherein cooking treatment and then mechanical defibration are carried out.

5. A process of making pulp according to claim 1, wherein mechanical defibration and then cooking treatment are carried out.

#### References Cited

##### UNITED STATES PATENTS

|           |        |                  |       |          |
|-----------|--------|------------------|-------|----------|
| 2,947,657 | 8/1960 | Peteri           | ----- | 162-76   |
| 3,382,140 | 5/1968 | Henderson et al. | ----- | 162-24 X |
| 3,446,699 | 5/1969 | Asplund et al.   | ----- | 162-28 X |
| 3,192,102 | 6/1965 | Nolan            | ----- | 162-24   |
| 3,467,574 | 9/1969 | West             | ----- | 162-71 X |

S. LEON BASHORE, Primary Examiner

A. L. CORBIN, Assistant Examiner

U.S. Cl. X.R.

162-28, 72, 84